

Feb. 7, 1961

W. UNSWORTH

2,970,904

INTRODUCTION OF ZIRCONIUM INTO MAGNESIUM

Filed April 27, 1959



INVENTOR

WILLIAM UNSWORTH

BY

Almon S. Nelson  
ATTORNEY

## 1

2,970,904

## INTRODUCTION OF ZIRCONIUM INTO MAGNESIUM

William Unsworth, Clifton Junction, near Manchester, England, assignor to Magnesium Elektron Limited, Clifton Junction, near Manchester, England, a company of Great Britain

Filed Apr. 27, 1959, Ser. No. 809,224

Claims priority, application Great Britain May 9, 1958

8 Claims. (Cl. 75—168)

This invention relates to the introduction of zirconium into magnesium and in particular to the production of a master alloy for introducing zirconium into magnesium especially for producing alloys of the kind defined in British Patent No. 511,137 which are substantially free from elements (which may be termed inhibitor elements) which combine with zirconium to form insoluble compounds in a molten magnesium melt, for example aluminium, silicon and iron, but may contain other elements (which may be termed "permissible elements") such as zinc, cadmium, thorium, rare earth metals, beryllium, indium, thallium, silver, copper, bismuth, lead and calcium. A small proportion of manganese can be tolerated. Another use for the master alloy is to precipitate iron or other inhibitor elements from magnesium.

It has been proposed in British Patent No. 652,222 to prepare such a master alloy consisting of three phases, viz. (1) a salt phase consisting of 1 to 30% by weight of the master alloy, (2) a matrix phase consisting of magnesium with or without permissible elements and zirconium, and (3) a zirconium rich phase embedded in the matrix phase. It was indicated that the salt phase might consist of various fluorides and/or chlorides. It was further known from British Patent No. 652,227 that when using alkali metal fluozirconate as the source of zirconium this must be mixed with some proportion of alkali metal chloride in order to avoid explosion when reacting with magnesium. It was found however that master alloys produced by this process were not metallic in appearance and contained at least 15 percent (and usually about 25 percent) of the salt phase with the disadvantage that an undue proportion of magnesium became trapped in the salt and so lost. This difficulty can be overcome by using zirconium fluoride instead of fluozirconate and a salt phase consisting wholly of fluorides, but this involves the use of lithium fluoride, which is very expensive, in order to achieve a sufficiently low melting point. The amount of the salt phase may also be controlled by using zirconium chloride instead of fluozirconate as described in British Patent No. 652,222, salt phase contents below 10% being fairly readily achieved and the alloy being more or less of metallic appearance. Zirconium chloride is however volatile, deliquescent, and readily hydrolysed therefore unpleasant to use and difficult to store. Furthermore, master alloys made from it show variations in alloying properties and the resulting alloys do not always fully exhibit the high tensile properties expected of the megnesium zirconium alloys.

The high salt residue content which arises when using fluozirconate was found to be due to the fact that the chloride residues are inspissated by the magnesium fluoride produced during the reaction with magnesium, as a result of which the chloride residue is not sufficiently fluid to enable it to be readily squeezed out of the master alloy. Since magnesium fluoride is known to be insoluble in alkali metal chlorides, and since mere dilution of the megnesium fluoride with excess of the chloride salts was not found effective, it has for some years been con-

## 2

sidered that the difficulty could not be overcome. The general insolubility of  $MgF_2$  in mixtures of alkali and alkaline earth chlorides is, moreover, well borne out by the literature and by its use to inspissate all manner of chloride-based fluxes for use with magnesium alloys. The inspissating effect of  $CaF_2$  in fluxes based on  $MgCl_2$  is itself a reflection of the insolubility of  $MgF_2$  in such chloride mixtures. On the other hand, since the unit of zirconium was cheaper in potassium fluozirconate than in zirconium chloride, and the fluozirconate was non-volatile, stable in air and readily stored and handled, it was very desirable commercially that the problem of preparing a master alloy with low salt content from fluozirconate should if possible be solved.

15 The present invention is based on the discovery that the problem can in fact be solved by providing in the reaction mixture a considerable excess of magnesium chloride in quantity sufficient (a) to react with all of the  $KF$ , (b) to react with all the  $ZrF_4$ , and (c) to provide 20 in addition enough unreacted magnesium chloride to dilute the alkali metal chlorides to such an extent and to establish such a high concentration of magnesium chloride in the salt phase that the magnesium chloride can largely dissolve the magnesium fluoride produced during the 25 reaction in spite of the alkali metal chlorides present, whereby the salt phase remains fluid and can be pressed out of the master alloy so as to leave a maximum of 10 percent salt phase in the master alloy and usually about 3 to 5 percent. The final master alloy is thus at 30 least as free from entrained salts as that made from chloride salt mixtures based on zirconium chloride.

Owing to the slightly inspissating effect of the residual  $MgF_2$  in the salt phase, the latter tends to be present in a few comparatively large inclusions in the interior 35 of the blocks or ingot into which it is cast, rather than to be widely distributed in small inclusions throughout the mass and spread out in thin films on the metal surface as is the case with master alloy made from the chloride. The master alloy of the present invention is 40 therefore of good metallic appearance and its keeping properties are markedly superior to those of chloride based master alloys.

Based on the above considerations the present invention provides a novel method of producing a master 45 alloy and a novel master alloy composition.

According to the invention a method for the production of the master alloy comprises heating together the following substances in the proportions stated, viz:

Alkali metal fluozirconate — 1 mol.  
50  $MgCl_2$  ————— 4.5 to 7.5 mols.  
Alkali metal chloride ————— 2.0 to 5.5 mols.  
Magnesium metal ————— 7 to 12 gram-atoms to 1  
gram/mol fluozirconate.

55 The alkali metal fluozirconate is preferably potassium fluozirconate having a ratio of  $KF$  to  $ZrF_4$  of from 1.0 to 2.0, viz.  $KZrF_5$  to  $K_2ZrF_6$ .

The alkali metal chloride is preferably  $KCl$  and/or  $NaCl$ .

The magnesium metal may be added in two stages, viz: 60 3 to 5 gram-atoms to 1 mol of fluozirconate in the first stage to produce a fairly stiff reaction product from which most of the salt residue can be readily expressed, the remainder being then added so as to make a master alloy which is sufficiently fluid to permit its being poured out of the crucible.

If less than 3 gram-atoms of magnesium is used in the first stage the zirconium forms a clinker-like mass and is not taken into solution even when more magnesium is added subsequently and if more than 5 gram-atoms is 70 used in the initial reaction a proportion of the magnesium may be lost with the salt residue.

If desired, some  $\text{BaCl}_2$  may be included in the reaction mixture in proportion up to 1.5 mols in order to suppress residual flux contamination in the final magnesium-zirconium alloy.

It is not generally desirable that any other ingredients should be included in the reaction mixture but it is possible also to include permissible elements other than calcium, e.g. replacing up to 60 percent of the magnesium. Beryllium however will not be incorporated in the magnesium in amounts exceeding 0.01 percent by weight of the mixture. Reducible chlorides of permissible elements may also be included in the reaction mixture, e.g. up to 50 percent of the  $\text{MgCl}_2$  can be replaced by an equivalent weight of thorium chloride or rare earth metal chloride.

Also according to the invention a 3-phase master alloy is produced having the following composition:

(1) A salt phase consisting of 1 to 10 percent by weight of the master alloy and containing  $\text{MgCl}_2$  and  $\text{MgF}_2$ , the latter being from 25 to 40 percent by weight of the  $\text{MgCl}_2$ , together with alkali metal chloride in quantity by weight from one-third to two-thirds the weight of the  $\text{MgCl}_2$ , with or without  $\text{BaCl}_2$ .

(2) A matrix phase consisting wholly or mainly of magnesium with or without zirconium and/or permissible elements.

(3) Metallic zirconium embedded in phase (2) and constituting 25 to 45 percent by weight of the master alloy.

The quantity of  $\text{BaCl}_2$  preferably does not exceed half the weight of  $\text{MgCl}_2$  in the chloride added for the initial reaction. The quantity of  $\text{BaCl}_2$  in the final master alloy, therefore, does not exceed twice the weight of the  $\text{MgF}_2$ . The presence of  $\text{BaCl}_2$  assists avoidance of flux particles in the final alloy but too much would unduly increase the melting point of the chloride phase used in the initial reaction which is preferably from 420°-600° C.

A particularly desirable range of chloride salt mixtures for the initial reaction is indicated by the area marked A in the accompanying drawing while the area marked B is preferred.

An example of the method of making the master alloy is as follows:

A mixture consisting of 374 lb.  $\text{MgCl}_2$ , 150 lb.  $\text{KCl}$  and 136 lb.  $\text{BaCl}_2$  was melted and added to 160 lb. of potassium fluozirconate in a separate crucible. The resulting mixture was heated to 650° C.: at this temperature 65 lbs. of solid preheated magnesium was added and when molten the melt was stirred to bring about the reaction. During stirring, the temperature of the melt rose to 800° C. owing to the strongly exothermic nature of the reaction between magnesium and the  $\text{ZrCl}_4$  formed in situ by the reaction of  $\text{MgCl}_2$  and  $\text{KZrF}_5$ . The chlorides were decanted away from the pasty zirconium master alloy in the bottom of the crucible. The master alloy was "pressed" to exclude the entrained chloride-fluoride phase and a further 65 lbs. of magnesium was added to dilute the master alloy to a consistency suitable to enable it to be cast into moulds. This melt yielded 165 lb. of zirconium master alloy containing 35 percent zirconium and 3.6 percent chloride.

Experience has shown that the master alloy of the present invention is constant in its alloying properties and gives consistently magnesium zirconium alloys with maximum tensile properties.

Another and unexpected advantage of the product over the corresponding chloride master alloy is its uniformity when molten. When preparing chloride based master alloy containing, for example, 30 percent zirconium, the mass of pasty alloy in the crucible readily separates into an upper fluid and a lower pasty layer on standing, necessitating stirring before casting each block. Segregation of zirconium can also occur in the blocks or ingots into which the master alloy is cast. The fluoride based master alloy of the present invention is however remarkably homogeneous and shows little tendency to segregate in the

molten state. This valuable property is illustrated by the following zirconium contents from the top and bottom of ingots of chloride based master alloy sold commercially and applicant's fluoride based master alloy.

| Master Alloy type                                          | Zirconium Contents |         |        |
|------------------------------------------------------------|--------------------|---------|--------|
|                                                            | Average            | Top     | Bottom |
| Commercial chloride based                                  | 30                 | 0.3/7.2 | 36.4   |
| Fluoride based in accordance with<br>Applicant's invention | 35                 | 39.0    | 37.3   |

As is well known small amounts of persistent zirconium chloride contamination are encountered in magnesium zirconium alloys made using chloride based master alloys, except in the case when the chloride salt phase of the master alloy is weighted with  $\text{BaCl}_2$  in accordance with the teaching of British Patent No. 652,230.

Experimental tests have confirmed that alloys made with applicant's master alloy are free from much residual chloride contamination.

I claim:

1. A method for the production of a master alloy suitable for introducing zirconium into magnesium, comprising heating together the following substances in the proportions stated:

Alkali metal fluozirconate 1 mol.  
 $\text{MgCl}_2$  4.5 to 7.5 mols.  
 $\text{Alkali metal chloride}$  2.0 to 5.5 mols.  
 $\text{Magnesium metal}$  7 to 12 gram-atoms to 1 gram/mol fluozirconate.

to a temperature above the melting point of magnesium.

2. A method as claimed in claim 1 wherein the fluozirconate is potassium fluozirconate having a ratio of  $\text{KF}$  to  $\text{ZrF}_4$  between 1.0 and 2.0.

3. A method as claimed in claim 1 wherein the alkali metal chloride is at least one chloride selected from the group consisting of potassium chloride and sodium chloride.

4. A method as claimed in claim 1 wherein the magnesium metal is added in two stages in which 3 to 5 gram-atoms to 1 mol fluozirconate in the first stage and the remainder after expressing most of the salt residue.

5. A method as claimed in claim 1 wherein some  $\text{BaCl}_2$  is included up to 1.5 mols.

6. A method as claimed in claim 1 wherein up to one-third of the magnesium is replaced by at least one of the elements, zinc, cadmium, thorium, rare earth metals, indium, thallium, silver and beryllium, the beryllium however not exceeding 0.01 percent.

7. A method as claimed in claim 1 wherein up to 50 percent of the  $\text{MgCl}_2$  is replaced by a chemically equivalent weight of at least one of the chlorides of the elements thorium, rare earth metals and manganese.

8. A master-alloy for introducing zirconium into magnesium comprising

a salt phase consisting of 1 to 10 percent by weight of the master alloy and containing  $\text{MgCl}_2$  and  $\text{MgF}_2$ , the latter being from 25 to 40 percent by weight of the  $\text{MgCl}_2$ , together with an alkali metal chloride in quantity by weight from one-third to two-thirds the weight of the  $\text{MgCl}_2$ ,

a matrix phase consisting substantially of magnesium, and at least one of the elements zirconium, zinc, cadmium, thorium, rare earth metals, indium, thallium, beryllium and silver,

and metallic zirconium embedded in said matrix phase and constituting 25 to 45 percent by weight of the master alloy.

References Cited in the file of this patent

UNITED STATES PATENTS

75 2,497,530 Ball et al. Feb. 14, 1950